

No. 879,530.

PATENTED FEB. 18, 1908.

L. DURAND.

PROCESS FOR THE REDUCTION OF COPPER ORE.

APPLICATION FILED JAN. 12, 1907.

FIG.1.



FIG.2.



FIG.3.



WITNESSES:

James Johnson  
M. A. Barret.

INVENTOR

Louis Durand  
Starvoostigher  
his ATTORNEY

FIG.4.



# UNITED STATES PATENT OFFICE.

LOUIS DURAND, OF DUMONT, NEW JERSEY, ASSIGNOR OF ONE-FIFTH TO RUBEN O. CURRIE,  
OF NEW YORK, N. Y.

## PROCESS FOR THE REDUCTION OF COPPER ORE.

No. 879,530.

Specification of Letters Patent.

Patented Feb. 18, 1908.

Application filed January 12, 1907. Serial No. 351,931.

To all whom it may concern:

Be it known that I, LOUIS DURAND, a citizen of the United States of America, residing at Dumont, in the State of New Jersey, have 5 invented certain new and useful Improvements in Processes for the Reduction of Copper Ore, of which the following is a specification.

My invention relates to a process for the 10 reduction of copper ores to a metallic state and it consists in first reducing said ores to a spongy state and then melting same and separating the pure molten copper from its associated products.

15 In order to explain my process and invention more fully and more particularly I will proceed to describe it in connection with the accompanying drawings which show an apparatus in which my said process can be carried into practical effect.

In these drawings Figure 1 represents a vertical section of said apparatus. Fig. 2 is a detail view on the line 2—2 of Fig. 1; Fig. 3 is a detail view of a grate which I employ in 25 said apparatus; Fig. 4 is a detail vertical section of the same parts shown in Fig. 1, with grate in position.

In these drawings, 1 represents a furnace having a compartment 2, for the reception of 30 the copper ore, sealed at the top by means of the following structure: At 3 is a pocket, square in shape, having at the bottom thereof a rubber or other pad 4 and a hood or cover 5 arranged to enter the pockets 3 and 35 to rest upon the pad 4, water being provided as shown to effect a sealing. The hood or cover 5 can be raised or lowered by means of a chain 6 connected with the hood or cover 5, at 7, the said chain moving on a pulley 8 and provided with a counter-poising or balancing weight 9. When it is desired to 40 provide a new supply of ore to the compartment 2, the hood or cover 5 is raised in the manner described and the ore can be introduced and thereafter the hood or cover can be brought down and the seal, as shown, can be effected.

At 10 I show a channel for receiving and retaining the grate 11 when it is desired to 50 insert the latter for the purpose of sustaining the copper ore above the line of said channel 10 so that the copper sponge can be removed from beneath the same. The grate 11 consists of a number of prongs 12 having a connecting web 13 near their outer ends the said

prongs being flat on the top and coming to a point or apex at the bottom and having a frame 14 cast integrally therewith and a rack 15 located centrally of the frame 14. A chain 16 is provided attached to the frame 14 at a point 17, the said chain 16 being suspended and traveling on the pulley 18.

When it is desired to introduce the grate into the ore chamber 2 it is let down from the position shown in Fig. 1 and brought to a horizontal position so as to occupy a line parallel with the channels 10. For the purpose of manipulating the same I provide ways 19 which support the grate while it is being forced into the chamber 2, and I also provide a pinion 20 operable by a shaft 21. The pinion 20 intermeshes with the rack 15 and forces the grate into the ore chamber and brings it to the position shown in Fig. 4, the cap 22 having been previously removed to permit the introduction of the grate. I also provide a pocket 23 which is adapted to catch any copper sponge which may accidentally stick to the grate 14 during its withdrawal. A cap 24 on the outer end of the 50 pocket 23 is provided so as to permit the removal of any copper sponge which may come into the pocket.

When the parts are in the position shown in Fig. 4 the grate 11 interposes a barrier 55 between the elements which I now desire to withdraw from the compartment 2 and those which I wish to retain therein for further action. The elements which I wish to detain in the compartment 2 lie above the grate and 60 those which I wish to withdraw are located below.

At 26 I provide a port having a door 25. By opening the door 25 a rabble may be introduced into the port 26 the copper sponge 95 and other elements lying underneath the grate 11 are pushed into the succeeding chamber hereinafter described. The door 25 is hung by a link 27 on a crane 28 the latter being suspended at points 29 to the frame of the 100 structure and a pillar 30 is provided for receiving the door when the copper sponge is being thus removed, and a handle 31 upon the door provides means for its easy manipulation.

At 32 I show a chamber for the reception of the fuel preferably wood charcoal, which produces the reducing agent. The chamber 32 is divided by the wall 33 into the chambers 34 and 35 and it is provided with an 110

upper extension 36 which affords means for storing the charcoal before it is introduced into the chamber 32. It is provided with a sealing device similar to the sealing device of 5 the ore chamber 2, and the reference letters employed in describing one sealing device is applicable to, and correctly describe, the other sealing device.

At 37 I provide a trap door which holds 10 the charcoal in the chamber 36, the said door being hinged at 38 to the frame work. A handle 39 is provided and a spring bolt 40 which can enter upper and lower notches 41 of the segment 42 and maintain the said trap 15 door in the closed position shown in Fig. 1, or in an open position. Twyers 43 are provided which introduce heated air into the chambers 34, 35, at the bottom thereof and through the openings 44. I secure this heated 20 air from a heating chamber (not shown), and I utilize the gases arising in the ore chamber 2 by drawing them off through a pipe 45 and leading them by means of a pipe 46 to the said air heating device (not shown), 25 for assisting in the creation of the heat in the said heat generating device.

At 47, I show a channel leading from the chambers 34, 35, and at 48 I show a reverberatory chamber into which the copper 30 sponge and its associated elements enter after they are thrust from the chamber 2 by way of the port 26. When the heated air enters the chambers 34, 35, and comes in contact with the body of the wood charcoal in 35 said chambers, the oxygen of the air combines with said charcoal and forms a mixture of CO and CO<sub>2</sub> in about equal proportions; the body or bed of charcoal is brought to and maintained at a state of incandescence, and the size or volume of this bed is 40 so fixed or proportioned that the result will be as aforesaid a mixture of CO and CO<sub>2</sub> in substantially equal proportions; this mixture passes into the reverberatory chamber 45 or furnace 48 where the copper sponge is melted; the temperature of the gases entering the chamber 48 being at melting heat; the gases escaping from this chamber after the melting of the copper sponge have a lower 50 temperature, but they have retained all of their reductive powers and have the proper temperature to convert copper ore into copper sponge. The heat produced by the generation of this mixture of gases is strong 55 enough to melt the copper sponge which is in the chamber of the reverberatory furnace 48 and the balance of the gaseous mixture has heat enough, when it reaches the chamber 2, to reduce the copper ore to the spongy state and 60 any iron contained in the ore to protodox of iron. The time required for the fusion of the material introduced into the reverberatory furnace is practically the same as that used for the reduction. When the melting 65 point is reached the protodox of iron being

fluxed with appropriate material, (say silica), a fusible silicate of iron is produced which rises to the top of the bath of molten metal with the slag and may be skimmed out. In this way the pure red metallic copper may be extracted from the melting chamber without any further operation. A gate 49 is shown for withdrawing the molten copper and gates 50 for withdrawing the slag.

By means of the apparatus above described wherein both the copper sponge and the copper ore are treated at the same time with reductant gas at proper temperatures double the metal can be produced per day as the reduction is at the same time as the 75 melting; there is therefore no loss of time in making the copper sponge and melting it. I take out one ton of molten metal made from copper sponge and then introduce another ton of copper sponge from the chamber 2 which is ready to go in, so every six hours I have one ton, or two tons, etc. according to the capacity of the apparatus. A mixture of CO and CO<sub>2</sub> giving really a heat generation of sufficient high temperature to heat 80 and melt any copper sponge and losing some of their heat at the further end of the chamber 48 the gases possess a lower temperature as they pass into the ore reducing compartment 2. A mixture of equal quantities of 85 carbonic oxide (CO) with carbonic acid gas (CO<sub>2</sub>) is reductant enough to extract 8% of oxygen from the peroxid of iron in the ores and bring the same to a state of protodox containing 22% of oxygen and it is also reductant enough to bring copper ore to a state 90 of metallic sponge.

In my present invention and by this process I produce a steady current of a mixture of CO and CO<sub>2</sub> with original melting temperature of generation passing through a reverberatory furnace where the copper sponge is melted; the gases, after their temperature has been reduced during the melting of the copper, pass to the compartment 105 containing the copper ore to be reduced to copper sponge. The peroxid of iron contained in the ore is reduced to protodox and cannot mix with the copper in the melting furnace and a flux being applied to it, (say 110 silica) a silicate of iron is formed which is fusible and which comes to the surface of the bath and is skimmed out with the slag.

It is to be noticed that the gases previously entering the reverberatory furnace at 115 melting heat do not lose any of their inherent reducing properties during the melting of the copper since the gas merely acts as a heating agent, the copper being already in a reduced state. The gases arrive at the reduction chamber with their reductant qualities unimpaired.

More particularly the operation of my process in the said apparatus is as follows: The ore to be reduced is introduced at the 120

top of chamber 2 the sealing device being temporarily removed for that purpose. The heated air in the meantime has been introduced through the twyers 43 and is being forced through the body of charcoal in the chambers 34, 35. This body of heated air in passing through the charcoal is resolved into  $\text{CO}_2$  and  $\text{CO}$  and nitrogen and arrives in the reverberatory chamber 48 at a temperature having heat units sufficient to bring the copper sponge in the reverberatory chamber to a molten condition are subtracted and the gases pass on and out of the reverberatory chamber into the chamber of reduction at a lower temperature and with their reducible qualities unimpaired. It is a matter of great economy and of high commercial importance that I am enabled to use the gases first for heating and melting and subsequently for reduction.

In carrying my process into effect also it will be seen that I apply reducing agents to the ore in the form of gases only: I have found that the direct application of fuel other than in the gaseous form prevents the formation of copper sponge.

In carrying my invention into effect also I apply these gases to the copper ores at a reducible temperature. A temperature largely in excess of this operates with such rapidity that it transforms the ore directly from its primal state into a state of pasty or muddy fusion. It is the special design of my present invention to obviate such an action.

Having thus described my invention, the following is what I claim as new therein and desire to secure by Letters Patent:

1. The process for reducing copper ore which consists in subjecting copper sponge to the action of a reducible gas at a melting temperature, thereby melting the sponge and at the same time reducing the temperature of the gas, and utilizing the gas at its reduced temperature to make more copper sponge.

2. The process of treating copper ore which consists in reducing the copper in the ore to a spongy condition, melting the sponge by means of a reducible gas at a high temperature, the gas being thereby lowered in temperature and reducing further amounts of copper ore by said gas at its lower temperature.

3. The process of reducing copper ores which consists in first reducing the copper in the ore to copper sponge, then withdrawing the said copper sponge into a separate chamber, adding a proper flux and bringing the copper sponge to a molten condition, and finally withdrawing the molten copper and the slag by separate means.

4. The process of reducing copper ores which consists first in reducing the copper in

the ore to copper sponge, then drawing off the copper sponge and other products associated therewith from the bottom of the reduction chamber and introducing them immediately therefrom into another chamber, and bringing the copper sponge to a molten state by gases passing therethrough to the reduction chamber.

5. The process hereinbefore described of first reducing the copper in the ore to copper sponge by means of reducible gases and then immediately bringing the same to a molten condition by means of gases at a melting temperature.

6. The process of reducing copper ores which consists in generating carbonic oxide and carbonic acid gas from the same body of charcoal, conducting said gases to a compartment containing copper ores, bringing said copper ores to copper sponge, then withdrawing said copper sponge into a separate chamber and bringing it to a molten condition and finally withdrawing the molten copper and other products separately.

7. The process of producing metallic copper from copper ores which consists in subjecting the ore to a reducible gas at a suitable temperature which will reduce the copper ore to copper sponge, and the iron in the ore to protoxide of iron, and then bringing the copper sponge to a molten condition.

8. The process hereinbefore described of bringing copper ore to a metallic and molten state by means of a single body of gases which first melts the copper already reduced and then passes to the reduction chamber for reduction purposes at a proper temperature and with its reducible qualities unimpaired.

9. The process substantially as hereinbefore described for bringing copper ore to a metallic and molten state through the operation of the following sequential acts, first, passing a blast of hot air through a bed of charcoal so arranged as to produce resulting gases of which 50% is carbonic oxide and 50% carbonic acid gas, second, passing said resultant gases through a chamber containing copper sponge and other products of a copper ore reduction chamber whereby the copper sponge is brought to a molten condition, third, conveying the said gases with their temperature lowered but with their reducible qualities unimpaired to the reduction chamber, and, fourth, reducing the copper ore in the reduction chamber to copper sponge by means of said gases.

This specification signed and witnessed this 31st day of December A. D., 1906.

LOUIS DURAND.

Signed in the presence of—

RUBEN O. CURRIE,  
HERBERT KNIGHT.